

# UNITED STATES PATENT OFFICE.

TENNEY L. DAVIS, OF SOMERVILLE, MASSACHUSETTS.

## HIGH EXPLOSIVE AND PROCESS OF PREPARING THE SAME.

1,419,027.

Specification of Letters Patent. Patented June 6, 1922.

No Drawing.

Application filed April 16, 1921. Serial No. 462,031.

(FILED UNDER THE ACT OF MARCH 3, 1883, 22 STAT. L., 625.)

To all whom it may concern:

Be it known that I, TENNEY L. DAVIS, a citizen of the United States, and a resident of Somerville, county of Middlesex, and 5 State of Massachusetts, have invented an Improvement in High Explosives and Processes of Preparing the Same, of which the following is a specification.

The invention described herein may be 10 used by the Government, or any of its officers or employees in prosecution of work for the Government, or by any other person in the United States, without payment to me of any royalty thereon.

15 The subject of this invention is a high explosive and process of preparing the same.

The main object of the invention is the production of a high explosive from naphthalene and the use of mercury nitrate as a 20 reagent in the nitration of naphthalene.

Naphthalene provides an abundant raw 25 material for the preparation of high explosives. The most powerful explosive which has heretofore been prepared from it is tetranitronaphthalene (containing 18.18% nitrogen) which, while not as powerful as trinitrotoluene or picric acid, has nevertheless found some use, alone or in a mixture, as a filling for high explosive shells.

30 I have discovered that the use of mercury nitrate as a reagent in nitration of naphthalene leads to the production of nitronaphthalenes. Naphthole nitrates more readily than naphthalene itself and I have succeeded in 35 preparing by this method explosives which contain more nitrogen than tetranitronaphthalene and which are more powerful.

While I have worked out a satisfactory process for the preparation of this explosive, I 40 do not desire to make the details of that process the object of the present application. I do, however, consider myself the inventor or discoverer of the general use of mercury nitrate as a reagent for the preparation of 45 high explosives from naphthalene. The explosive which is produced by this process is a crude pentanitronaphthole which substance I also claim as my invention or discovery.

50 The process may be carried out as follows:—

I describe the two step process though the process may equally be carried out in one step or in three. 10 kilograms of naphtha-

lene is treated, with stirring, with 30 liters 55 of commercial nitric acid (specific gravity 1.42) in which half a kilogram of mercury nitrate has been dissolved and the mixture is melted until red fumes begin to come off abundantly. This occurs at about 75° C., 60 and the mixture is kept at 70 to 80° C. until the vigorous evolution of gas has subsided. The spent acid contains the mercury nitrate and may be fortified and used again for the first step of the process. The oil contains 65 about 8.9% of nitrogen and consists largely of nitronaphthalenes together with a small quantity of nitronaphthalenes. This oil is submitted directly to the second step of the nitration. While stirred and cooled, it is 70 treated with 82.4 liters of concentrated sulphuric acid (specific gravity 1.82). 100 liters of nitric acid (specific gravity 1.49) is then added. A vigorous reaction takes place, copious red fumes are evolved and it 75 is necessary to cool the reaction mixture. When the evolution of red fumes has subsided the mixture is heated for an hour at 110° to 115°. It is then allowed to stand over night and the crystals of pentanitro- 80 naphthole which have separated are filtered off from the strongly acid liquid by means of an asbestos or filtrose filter. The pentanitronaphthole which is so obtained is purified in the usual way by boiling with 85 water. It is an almost colorless crystalline substance which does not melt but decomposes at about 257°. It contains about 19% nitrogen and has the acidic properties which are characteristic of nitrophenols. When 90 the spent acids from the second step of nitration are diluted with water, a yellowish orange mass is precipitated. This material melts at from 60° to 105° and consists of the lower nitronaphthalenes together with a 95 quantity of nitronaphthalenes. It contains about 17.7% of nitrogen, and may be used as a high explosive alone or in mixtures.

Having described my invention what I claim as new and desire to secure by Letters Patent, is:

1. The method of preparing pentanitronaphthole, comprising treating naphthalene with a mixture of nitric acid and mercury nitrate to produce nitronaphthalenes, treating the nitronaphthalenes with sulfuric acid, treating the mixture with nitric acid, filtering the resultant mixture to recover the crystals of

pentanitronaphthole and purifying the pentanitronaphthole.

2. The method of preparing pentanitronaphthole, comprising nitrating naphthalene, recovering the resulting nitronaphtholes, nitrating the nitronaphtholes and then removing the pentanitronaphthole.

3. The method of preparing pentanitro-

naphthole, comprising nitrating naphthalene and then removing the resulting pentanitronaphthole.

4. A new article of manufacture, consisting of pentanitronaphthole.

5. A high explosive consisting of pentanitronaphthole.

TENNEY L. DAVIS.